

March 1, 1938.

E. G. GRUNDSTROM

2,109,530

METHOD AND MEANS FOR MAKING CASTINGS

Filed July 10, 1937.



Inventor:  
Erik G. Grundstrom,  
By Wilkinson, Hulley, Byron & Knight  
Atty.

## UNITED STATES PATENT OFFICE

2,109,530

METHOD AND MEANS FOR MAKING  
CASTINGSErik G. Grundstrom, Chicago, Ill., assignor to  
Advance Aluminum Castings Corp., Chicago,  
Ill., a corporation of Illinois

Application July 10, 1937, Serial No. 152,882

3 Claims. (Cl. 22—200)

The present invention relates to methods and means for making castings.

In making certain castings, particularly those having long, relatively thin sections, it has been difficult to maintain the molten metal in pure condition as it enters the mold and to obtain a perfect casting. This difficulty has been encountered to a very considerable extent in making castings of aluminum or aluminum alloys; the dross having a tendency to enter the mold cavity.

An object of the present invention is to provide improved apparatus for making castings, particularly for making castings of aluminum or alloys thereof.

A further object is to provide an improved method for making castings in which dross, oxides and the like are prevented from entering the mold cavity.

Further objects will appear as the description proceeds.

Referring to the drawing—

Figure 1 is a sectional view of a two-part mold embodying the principles of the present invention, said figure being taken along the plane indicated by the arrows 1—1 of Figure 2;

Figure 2 is a view taken along the plane indicated by the arrows 2—2 of Figure 1, half of the mold being removed; and

Figure 3 is a sectional view taken along the plane indicated by the arrows 3—3 of Figure 1.

A two-part mold of the permanent mold type is illustrated in the drawing. Said mold includes the two cooperating mold parts 10 and 11, said mold parts having cooperating faces to mold a casting such as indicated by the numeral 12. The particular casting chosen for illustration is the head of the motor of an internal combustion engine. Said casting is long and rather wide but relatively thin in most of its cross section. Many difficulties have been encountered in the past in making such a casting due to the fact that the molten aluminum or aluminum alloy must under usual practical conditions drop through a considerable distance, collecting air and forming dross, oxides and the like. Considerable difficulties have been encountered in preventing dross and the like from entering the mold cavity.

The mold cavity for forming the casting 12 is indicated by the numeral 13, said cavity being formed by the cooperating faces of the two mold parts 10 and 11. Said mold parts are formed to provide a gate, indicated by the numeral 14, which gate is an elongated cavity. As the parts

erably be vertically disposed. The two parts 10 and 11 of the mold are provided with grooves for the reception of a strainer, indicated by the numeral 15. Said strainer is an elongated member provided with holes 16 throughout the greater part of its length. The upper extremity of the strainer 15 is bent over to provide a hand hold 17. Adjacent to the gate 14 is the inlet passage 18, through which molten aluminum or the like can be admitted to the gate 14. Said passage 18 and gate 14 have communication with one another adjacent to the lower extremity of said gate 14, the lower extremities of the gate 14 and the passageway 18 being connected by the passageway 19. Cross passageways 20—20 may be provided at various levels for the purpose of admitting molten metal at various heights along the gate 14. The strainer 15 may be made of steel or other material which will not be attacked by the molten aluminum or the like. For practical reasons the passage 18 has its length disposed substantially vertically.

In operation the strainer 15 will be located in position dividing the gate 14 from the mold cavity 13. As molten aluminum or the like is poured into the passage 18, said molten metal will rise in the gate 14 and will be strained through the strainer 15 into the mold cavity 13. The dross, or the like, which may form in the molten aluminum will be held back by said strainer 15 and only the pure metal will pass through the holes 16 into the mold cavity 13.

After the mold cavity has been filled and while the molten metal is quiescent and before the aluminum has solidified, the strainer 15 will be withdrawn. As the casting within the mold cavity 13 solidifies and shrinks in the solidifying process, metal will be drawn into said mold cavity from the gate 14 to compensate for said shrinkage, the necessary free access being had by reason of the withdrawal of the strainer 15.

Many modifications of the present invention will occur to those skilled in the art. It is intended to cover all such modifications that fall within the scope of the appended claims.

What is claimed is—

1. In a permanent mold, in combination, cooperating mold parts defining a mold cavity, said mold parts defining a passageway comprising a gate cavity for admitting molten metal to said mold cavity, and a strainer adapted to be positioned between said gate cavity and said mold cavity, said strainer being removable from between said gate cavity and said mold cavity while

metal in said gate cavity and said mold cavity is in unsolidified condition.

2. In a permanent mold, in combination, mold parts defining the mold cavity and a gate cavity 5 communicating with said mold cavity, said mold parts also having a passageway adapted to deliver molten metal simultaneously to various regions along said gate cavity, and a strainer adapted to be positioned between said gate cavity and 10 said mold cavity, said strainer being removable

when said mold parts are in cooperative relationship with each other.

3. The method of making a casting which consists of admitting molten metal to a mold cavity through a strainer, permitting said strainer to 5 remain in cooperative relationship with said mold cavity until the metal in said mold cavity is quiescent, and thereafter removing said strainer before said metal has solidified.

ERIK G. GRUNDSTROM. 10